

May 31, 1960

E. K. BAUER ET AL

2,938,256

METHOD AND APPARATUS FOR MAKING BULKED YARN

Filed March 6, 1957



1

2,938,256

## METHOD AND APPARATUS FOR MAKING BULKED YARN

Ernest K. Bauer, Meadville, and Wendell D. Shumaker, Saegertown, Pa., assignors to American Viscose Corporation, Philadelphia, Pa., a corporation of Delaware

Filed Mar. 6, 1957, Ser. No. 644,308

9 Claims. (Cl. 28—1)

The invention relates to the manufacture of bulky yarns and more particularly to a method and apparatus for producing a yarn of increased bulk by swirling or whipping the individual continuous and substantially straight filaments of a multi-filament yarn into convolutions or ring-like loops or coils of various sizes and at random intervals along the length of the yarn.

In the manufacture of artificial fibers, which are most usually produced as unbroken filaments, various procedures have been proposed in an attempt to produce a continuous yarn having the lightweight and fluffy character of a yarn spun from staple fibers. Until recently, the physical character of these continuous multi-filament yarns has been modified or distorted into a bulked condition by chemical treatments, either during or after the formation of the yarn itself, or by mechanical manipulations, as for example where the yarn is crimped or twisted or where the filaments thereof are broken by cutting or abrading the same. In general, these previous efforts resulted in a yarn which only temporarily retained its distorted or bulked character and, for the most part, involved a considerable sacrifice in the inherent strength characteristic of continuous multi-filament yarns. Accordingly, it is a primary object of this invention to provide an improved and generally more satisfactory method and apparatus for bulking continuous multi-filament yarns.

Another object is the provision of an improved method wherein the individual filaments of a continuous multi-filament yarn are separated from each other and swirled into convolutions or ring-like loops while being simultaneously advanced in a generally straight-line direction.

Still another object of the invention is to provide an improved method wherein the individual filaments of a continuous multi-filament yarn are separated from each other and swirled into a mass of snarled or entangled ring-like loops extending at random intervals along the length of the yarn by an expanding fluid stream, while simultaneously being advanced in an axial direction through a restricted area by the fluid stream itself.

A further object is the provision of an improved apparatus having a bulking chamber within which the individual filaments of a continuous multi-filament yarn are separated from each other and concomitantly swirled or whipped into a bulked or looped formation by an expanding fluid stream.

A still further object is to provide a more satisfactory yarn bulking apparatus within which a continuous multi-filament yarn is caused to alter its axial direction of travel while simultaneously being impinged with a turbulent stream of fluid to effect a haphazard or random looping of the filaments along the yarn length.

Yet, another object is the provision of a yarn bulking apparatus having a bulking chamber of non-uniform cross-section designed to disrupt a streamlined fluid flow into a turbulent flow which effects a vibratory separation of the individual filaments of a continuous multi-filament

2

yarn and a swirling of the same into ring-like loops at random intervals along the length of the filaments as the yarn of filaments travels continuously through the bulking chamber.

5 These and other objects and advantages of the invention will be apparent from the following description and accompanying drawing in which:

Figure 1 is a schematic view illustrating the bulking apparatus of the present invention in its manner of use;

10 Figure 2 is a plan view of one form of yarn bulking device of the present invention;

Figure 3 is an expanded view illustrating, in perspective, the parts of the yarn bulking apparatus shown in Figure 2;

15 Figure 4 is a vertical longitudinal section taken substantially along the lines 4—4 of Figure 2;

Figure 5 is an expanded view of a modified form of yarn bulking apparatus; and

20 Figure 6 is a fragmentary sectional view of a still further modified yarn bulking device of the present invention.

In general, the bulking of a continuous multi-filament yarn in accordance with the present invention is accomplished by passing the yarn through confined delivery

25 and bulking chambers or passages, into the latter of which is also introduced a jet of compressible fluid. The yarn delivery and bulking chambers provide a continuous yarn path through the device, but are disposed in laterally offset relationship, thus necessitating that

30 the yarn alter its direction of axial travel as it leaves the delivery chamber and enters into the bulking chamber. The compressible fluid, as for example air, is introduced into the bulking chamber along a course inclined at an acute angle to the general direction of yarn travel and substantially at the area in which the yarn alters its axial travel in moving from one chamber to the other.

With this structural arrangement, a streamlined flow of compressible fluid expands and is disrupted upon its entry into the bulking chamber, into a turbulent flow

40 which impinges against the yarn as it alters its axial course and enters into the bulking chamber. The impact and turbulence of the fluid serves to violently vibrate the yarn filaments apart from each other and swirl

45 or whip the same into a plurality of convolutions or ring-like loops which are randomly spaced along the length of the filaments and which become entangled with each other as the yarn continues its passage through the bulking chamber.

50 To maintain and reinforce the turbulent effect of the fluid stream on the yarn filaments passing through the bulking chamber, the walls of this chamber may be provided with longitudinally spaced projections which, in effect, serve as deflectors or obstructions for both the compressible fluid and the yarn passing

55 ing therethrough.

With reference to the drawing, Figure 1 illustrates a

60 yarn 11 consisting of a plurality of continuous substantially straight filaments supplied from a suitable source, not shown, and delivered into and through the yarn

bulking apparatus of the present invention, indicated

65 generally at 13. During its travel through the device

70 13, the yarn filaments are distorted into the desirable convoluted or looped formation as more fully described hereinafter, and are then passed over and through the guides 15, 17 and 19, between the take-up rolls 23 and 25, and collected on a conventional wind-up device schematically illustrated at 27. As the bulked or treated yarn passes onto the wind-up device, it is given a slight twist to assist in maintaining the filaments in their bulked condition. It will be understood that the degree of twist imparted to the bulked yarn may be varied as desired,

with the greater the twist, the more firmly the individual filaments are held together.

As shown in Figures 2-4, the bulking apparatus 13 includes yarn delivery and bulking chambers or passages 29 and 31, respectively, and a fluid delivery duct 33 interconnecting a fluid inlet opening 35 with the bulking chamber 31. For the sake of economy and ease in manufacture, the bulking apparatus 13 is formed of plates 37 and 39 releasably secured together by bolts 41, with their faces 43 and 45 in snug contact. If desired, a gasket, not shown, may be interposed between the plates 37 and 39 to assure a satisfactory fluid seal therebetween. As shown in Figure 3, the face 43 of the plate 37 is provided with a pair of substantially straight channels 47 and 49 which together form a continuous path extending between opposite ends of the plate 37. For purposes as described hereafter, the channel 47 is made deeper but narrower than the channel 49, and terminates within the channel 49 as shown at 51. In a similar manner, the face 45 of the plate 39 is grooved to form generally straight channels 53 and 55, the latter of which extends at an angle of approximately 30° to the axis of the channel 53. From the structure thus far described, it will be seen that the respective plates 37 and 39 can be easily machined with conventional equipment to provide the necessary channels therein. Further, while channels of rectangular cross-section have been illustrated, it will be understood that channels of other cross-sectional configuration may be employed if desired.

After this preliminary machining of the parts, the plates 37 and 39 are secured together by the bolts 41. In this assembled condition of the parts, the channels 49 and 53 are aligned with each other and together form the bulking chamber 31, while the channels 47 and 55 are closed by the adjacent smooth surfaces of the plates 39 and 37, respectively, to provide the yarn delivery chamber 29 and fluid delivery duct 33 heretofore noted. As seen particularly in Figure 4, the chambers 29 and 31 provide a continuous passage through the device. The axes of these chambers, however, lie along substantially parallel planes offset laterally from each other thus providing the continuous passage with an angulated portion which causes the yarn of filaments to alter its straight line course as it passes from the chamber 29 to the chamber 31. The duct 33 opens into the chamber 31 substantially in the area within which the yarn alters its course and the yarn filaments will therefore be subjected to the full impact of the compressible fluid delivered through the duct 33. Further, it will be noted that the enlarged cross-section of the chamber 31, as compared to the duct 33, permits a rapid expansion of the inrushing fluid and that the angular inclination of the duct 33 directs the fluid and yarn toward the exit of the chamber 31.

The inlet opening 35 is formed when the plates 37 and 39 are in their assembled condition, and is internally threaded to facilitate attachment of the hose 57 connected to a suitable source of compressible fluid, as for example air. In addition, the inlet area of the chamber 29 is countersunk as shown at 59 to facilitate lacing of the yarn thereto.

During the bulking process, the yarn of filaments 11 travels a generally straight-line path into and through the chamber 29 and then alters its course for movement into the bulking chamber 31. As heretofore mentioned, the yarn of filaments, during its change in course, intersects a blast of air or other compressible fluid flowing into the bulking chamber 31 through the duct 33. The expansion and impact of the fluid against the yarn serves to disrupt the same into a turbulent flow, which in turn effects a violent vibratory separation of the yarn filaments and a swirling of the same in a haphazard fashion into a plurality of convolutions or ring-like loops formed at random intervals along the length

of the filaments. In view of the turbulent condition of the fluid as it flows toward the exit of the bulking chamber 31, the initial ring-like loops formed in the filaments tends to become snarled or entwined with each other thereby locking the loops in place. From the procedure described, it will of course be apparent that the velocity of the compressed air is adjusted for the particular effect desired and may be even varied or delivered at a pulsating rate to form a novel yarn bulked at intermittent intervals. Further, it will be recognized that the yarn delivery and withdrawal rates must be so correlated to prevent the filaments from being pulled into their straight condition before the filament loops have become snarled or before the yarn is given a twist.

As heretofore mentioned, the compressible fluid or air delivered into the bulking chamber is maintained in its turbulent condition and perhaps made more turbulent as it flows toward the exit of this chamber to insure the desired bulking effect on the yarn filaments with a minimum of compressed air. This result is accomplished, for example, by the structure shown in Figure 5 which includes a pair of plates 137 and 139, corresponding to the plates 37 and 39 heretofore described. As shown, the plate 137 is formed with channels 147 and 149, while the plate 139 is provided with channels 153 and 155. When assembled by bolts extending through the openings 156, the channels 149 and 153 cooperate to form a bulking chamber or passage similar to the chamber 31, while the channels 147 and 155 are closed to provide a yarn delivery chamber or passage and a fluid delivery duct. The annular threaded portions 157 and 159 in each of the plates 137 and 139 of course are aligned when the plates are assembled and serve as an air inlet opening and enlarged entrance for the yarn delivery chamber in a manner as shown at 35 and 59, respectively, in Figure 2.

In this modified bulking apparatus shown in Figure 5, however, it will be noted that the periphery of the channels 149 and 153 are formed with longitudinally spaced projections 161 which, for the sake of ease in manufacture, may be screw threads cut after the plates 137 and 139 are assembled. As with the apparatus shown in Figures 2-4, the yarn delivery and bulking chambers of the structure shown in Figure 5 are substantially parallel and are laterally offset from each other so that the yarn filaments will undergo a similar vibratory separation and swirling into ring-like loops as it travels from the yarn delivery chamber to the bulking chamber. However, with the structure of Figure 5, the air or other compressible fluid flowing toward the exit of the bulking chamber as well as the yarn filaments, will strike the projections 161 and will accordingly be deflected from a straight-line path. This will of course prevent the air from resuming a streamlined flow through the bulking chamber and results in maintaining the desired turbulent air condition reacting against the yarn filaments during their travel toward the bulking chamber exit. With the apparatus shown in Figure 5, it will be apparent that maximum use is made of the compressed air and that the yarn treated with this device has a highly bulked character with the ring-like loops randomly spaced along the length of the filaments and entangled with each other.

The fragmentary view of the apparatus shown in Figure 6 is similar, both in function and construction, to the devices heretofore described, and includes yarn delivery and bulking chambers 229 and 231 and a duct 233 for use in delivery of air or other compressible fluid. As with the arrangement shown in Figure 5, the bulking chamber 231 is provided with longitudinally spaced projections 261 disposed in alternate relationship along opposite walls of the bulking chamber. In addition to maintaining the air in a turbulent condition, in a manner as described in relation to the apparatus of Figure 5, the projections 261 deflect both the air and yarn filaments

along a sinuous path to cause the filaments and air flow to repeatedly intersect each other as they travel through the bulking chamber.

It is seen that the above described process and apparatus effect a maximum bulking of the yarn filaments by subjecting the same, within a confined area, to a highly turbulent flow of compressed fluid or air. Further, it will be noted that the mode of yarn treatment described entails a highly efficient use of the compressed fluid while the apparatus is compact, simple and economical in construction and use.

It is seen from the above description that the objects of the invention are well fulfilled by the method and apparatus described. The description is intended to be illustrative only and it is to be understood that changes and variations may be made without departing from the spirit and scope of the invention as defined by the appended claims.

We claim:

1. A process for making bulky continuous filament yarn from a yarn of continuous substantially straight filaments including the steps of delivering the yarn of filaments through a first confined path and into a second confined path interconnected therewith, the axes of said first and second confined paths being in laterally offset relationship whereby the yarn of filaments is caused to alter its course of travel as it passes from said first confined path into said second confined path, and impinging a fluid stream against the yarn of filaments as it alters its course of travel and passes into the second confined path to separate the filaments and swirl the same into a plurality of ring-like loops spaced at random intervals along the length of the filaments.

2. A process as defined in claim 1 in which the fluid stream enters the second confined path at an acute angle to the general direction of yarn travel therethrough.

3. A process for making bulky continuous filament yarn from a yarn of continuous substantially straight filaments including the steps of delivering the yarn of filaments through a first confined path and into a second confined path interconnected with and spaced laterally from the first confined path, impinging a stream of fluid against the yarn of filaments as it passes into the second confined path to separate the filaments and swirl the same into a plurality of ring-like loops at random intervals along the length of the filaments, and maintaining the stream of fluid in a turbulent condition as it passes through the second confined path along with the yarn of filaments.

4. A process as defined in claim 3 in which the yarn of filaments is moved sinuously through the second confined path.

5. Apparatus for making continuous filament yarn from a yarn of continuous straight filaments including a bulking device having a continuous confined passage extending therethrough and opening at opposite ends thereof, said passage having a first substantially straight portion lying within a first plane and a second portion lying within a second plane disposed in substantially parallel and laterally offset relationship with respect to said first plane, said first portion opening into said second portion and providing a continuous path for the yarn of filaments from said first portion into said second portion, an inlet for introducing a stream of compressible fluid into said bulking device, and a duct extending from said inlet to said second portion of the passage for impinging the yarn of filaments with the stream of compressible fluid as the yarn enters said passage second portion.

6. Apparatus as defined in claim 5 wherein said duct extends at an acute angle to the direction of yarn travel from said first portion to said second portion.

7. Apparatus as defined in claim 5 wherein said passage second portion includes longitudinally spaced projections extending along its periphery.

8. Apparatus as defined in claim 7 wherein said projections are in the form of screw threads.

9. Apparatus as defined in claim 7 wherein said projections are alternately disposed along opposite longitudinal walls of said second portion to provide a sinuous path therethrough.

#### References Cited in the file of this patent

#### UNITED STATES PATENTS

|           |             |       |                |
|-----------|-------------|-------|----------------|
| 132,582   | Jenks       | ----- | Oct. 29, 1872  |
| 2,100,588 | Claus       | ----- | Nov. 30, 1937  |
| 2,423,721 | Nelson      | ----- | July 8, 1947   |
| 2,783,609 | Breen       | ----- | Mar. 5, 1957   |
| 2,852,906 | Breen       | ----- | Sept. 23, 1958 |
| 2,884,756 | Head        | ----- | May 5, 1959    |
| 2,911,784 | Vandervoort | ----- | Nov. 10, 1959  |
| 2,924,000 | Griset      | ----- | Feb. 9, 1960   |

#### FOREIGN PATENTS

|                                 |       |               |
|---------------------------------|-------|---------------|
| Australia                       | ----- | Feb. 10, 1955 |
| Germany                         | ----- | Feb. 1, 1929  |
| Belgium                         | ----- | Nov. 14, 1955 |
| France                          | ----- | Apr. 6, 1955  |
| France                          | ----- | Oct. 26, 1955 |
| (Corresponding Canadian patent) | ----- | June 2, 1959  |